

UNITED STATES PATENT OFFICE.

ELROY A. CHASE, OF NORTHFIELD, VERMONT.

## PROCESS OF TREATING THE SURFACE OF GRANITE OR LIKE STONE.

No Drawing.

Application filed July 30, 1925. Serial No. 47,158.

This invention relates to a process of treating the surface of granite or like stone, by which process new and very desirable results are obtained.

5 It is customary to use a sand blast for  
treating the surface of granite and particu-  
larly for producing letters and other designs  
thereon, the sand blast being commonly  
directed through a stencil, so that the back-  
10 ground is cut away by the sand blast below  
the original surface of the stone. In the  
cutting of such materials and particularly  
of light colored granite, it has been found  
very difficult to bring out a satisfactory  
15 contrast between the natural or unpolished  
surface of the stone and the surface pro-  
duced by the sand blast, particularly when  
sinking a design therein.

It is the object of my invention to provide a process of treating the surface of granite and like stone by which the portions subjected to the sand blast will acquire a different finish and appearance, so that the contrast with the remaining surface of the work will be more marked and the design will stand out more prominently therefrom.

The detailed steps of my improved process are hereinafter described and will be more specifically set forth in the appended claims.

30 In carrying out my improved process, I make use of an abrasive compound comprising a mixture of fine grains of sand with a certain proportion of fine grains of a hard abrasive material, such as carborundum or 35 silicon carbide.

The proportions of the mixture may be somewhat widely varied, an increased amount of the abrasive material producing more rapid cutting of the stone but at the same time increasing the cost of the mixture. The most desirable proportion to be used on a given piece of work depends upon a careful consideration and comparison of the cost of the mixture with the cost of the time and labor consumed in cutting the design.

I find that a very effective mixture consists of about one part of silicon carbide or carborundum and about one part of sand. The sand may be an artificial product having sharp or crystalline grains with a marked cutting action of its own, or it may consist of a fine sea sand in which the grains are small and rounded rather than crystalline. The artificial sand produces somewhat more

rapid results while for some purposes the **55** sea sand is very satisfactory.

The proportion of sand to carborundum may be substantially increased when it is desired to reduce the cost of the mixture and very good results may be obtained with two, three, or even four parts of sand to one part of carborundum. 60

When this abrasive mixture is used in cutting granite or like stone with a sand blast, I have found that the surface produced is distinctly and prominently darker in appearance and color than the surface produced by the use of sand alone. This darker color is not the result of discoloration or stain due to the carborundum or carbide, but appears to be caused by the abrasive action of the carborundum upon the stone, in addition to the usual action of the sand. The surfaces appear to be somewhat more smoothly finished and to have a certain degree of polish which is not found where sand alone is used as an abrasive.

While my improved process is particularly adapted for sinking a design below a previously finished surface of stone, it is also well adapted for finishing flat or irregular surfaces of stone and when thus used the finished stone is substantially darker in appearance than that produced by the usual sand blast with sand alone. 80 85

While I have used carborundum and silicon carbide as convenient terms for designating the abrasive to be mixed with the sand, it will be understood that other abrasives having similar characteristics may be substituted for use in my improved process and that their use comes within the scope of my invention as set forth in the claims. 90

Having fully described the steps of my improved process and the results and advantages thereof, I do not wish to be otherwise limited to the details herein disclosed but what I claim is:—

1. The process of treating the surface of granite or like stone which consists in sand blasting the stone with a mixture of fine grains of sand and fine grains of silicon carbide, each in substantial proportions. 100

2. The process of treating the surface of granite or like stone which consists in sand blasting the stone with a mixture of one to three parts of fine grains of sand and one part of fine grains of silicon carbide. 105

- 2
3. The process of treating the surface of granite or like stone which consists in sand blasting the stone with a mixture of a relatively large portion of small rounded grains of sand and a substantially smaller portion of fine grains of a hard abrasive polishing material.
  4. The process of treating the surface of granite or like stone which consists in subjecting the surface of the stone to the simultaneous action of sea sand and not more

than an equal portion of fine grains of hard abrasive directed as a sand blast against the surface of said stone.

5. The process of producing the effect of contrasting colors in granite or like stone, which consists in sand blasting part of the surface with a mixture of sand and fine grains of silicon carbide.

In testimony whereof I have hereunto affixed my signature.

ELROY A. CHASE.